

Aug. 29, 1944.

R. H. LOMBARD

2,356,938

VITRIFIED DIAMOND GRINDING WHEEL

Filed Jan. 6, 1942



FIG. 1



FIG. 2



FIG. 3



FIG. 4



FIG. 5

Inventor

ROBERT H. LOMBARD

By *George J. Deompson*  
Attorney

## UNITED STATES PATENT OFFICE

2,356,938

## VITRIFIED DIAMOND GRINDING WHEEL

Robert H. Lombard, Worcester, Mass., assignor  
to Norton Company, Worcester, Mass., a cor-  
poration of Massachusetts

Application January 6, 1942, Serial No. 425,803

4 Claims.

(Cl. 51—307)

The invention relates to vitrified diamond grinding wheels.

One object of the invention is to provide a technique for the manufacture of vitrified bonded diamond grinding wheels and sticks or hones which shall be as simple as possible and give consistently good results. Another object of the invention is to provide a structure for two-part vitrified diamond grinding wheels having an abrasive rim or periphery and a non-abrasive center, which structure shall be integral and can be duplicated with few, if any, rejections during manufacture.

Another object of the invention is to control and prevent swelling of either the center or the abrasive portion of a vitrified bonded diamond grinding wheel. Another object of the invention is to provide a mix for a center for such a wheel capable of being matured into a strong and uniform center in a vitrifying process. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein, and the scope of the application of which will be indicated in the following claims.

In the accompanying drawing illustrating one of many possible embodiments of the mechanical features of this invention,

Figure 1 is a cross sectional view of a mold having just been filled with a vitrified non-abrasive mix to form the center of a peripheral vitrified diamond grinding wheel;

Figure 2 shows the mold of Figure 1 with a top plate in position;

Figure 3 shows the mold of Figures 1 and 2 after pressing of the center, after inversion, after the mold ring has been removed and a two-diameter mold band placed outside of the largest mold plate;

Figure 4 shows the mold in the same condition as in Figure 3 after the annular space has been filled with diamond ceramic material and the ring reinserted; and

Figure 5 shows the mold of Figure 4 after it is closed.

The drawing illustrates the manufacture of a peripheral wheel. From this it should not be understood that peripheral wheels are more important or manufactured in greater quantities than cup wheels and others having an annular

plane abrasive surface because perhaps the reverse is the fact, but the manufacture of a peripheral ceramic diamond grinding wheel presents particular problems and from the following disclosure the manufacture of a diamond ceramic cup wheel will be readily understood. In the first place, it may be noted that owing to the great cost of diamonds, it is quite usual to make diamond grinding wheels in the form of a thin annulus of diamond abrasive with a non-abrasive center. A ceramic bonded diamond abrasive wheel has certain free-cutting and wear resisting properties which make it highly desirable for certain grinding operations. It is desirable to make a vitrified center for such diamond grinding wheels and in order to make an integral body free from cracks or strains, it is desirable to vitrify the center or back at the same time that the rim is vitrified.

20 Swelling is a particular problem and, therefore, it is important to provide a mix both for the center and the annulus which will not swell during firing. I shall first describe the steps in the molding technique for the production of a green body ready for firing in a suitable furnace.

Referring now to Figure 1, I provide a large flat plate 9 and a mold consisting of a plate 10, a ring 11, and an arbor 12. The ring 11 just fits the plate 10 and the arbor 12 just fits in a central hole 13 in the plate 10. I first place the plate 10 upon the plate 9 and at opposite sides of the plate 10 I position a pair of spacing blocks 14. I then place the ring 11 around the plate 10 and upon the blocks 14, as shown. I then insert 30 the arbor 12 part way into the hole 13. I now fill the mold with a center non-abrasive mix 15 and level it off in a well known manner.

I now transfer the filled mold of Figure 1 on the plate 9 to the bottom plate of a hydraulic press. Referring to Figure 2, I now place upon the arbor 12 a plate 16 having an arbor hole 17 and having a diameter somewhat greater than that of the plate 10. I now remove the blocks 14 and temporarily hold up the ring 11 with my fingers. Then I apply the pressure of the hydraulic press to the extent of about 250 pounds per square inch. After the ring 11 starts to move, sufficient grit moves between it and the plate 10 to prevent the ring 11 from dropping.

50 I now strip the mold ring 11 and invert the mold, locating the plate 16 on the bottom plate of the hydraulic press. A consolidated center mix 15a is now located between the plates 10 and 16. Then I place a heavy mold band 18 around the plate 16 and upon spacing blocks 19. The

mold band 18 has a small inside diameter approximately the same as that of the outside diameter of the plate 16 so as to fit upon it with a sliding fit. It has a larger inside diameter separated therefrom by a shoulder 21. When the band 18 is raised by the blocks 19, the shoulder 21 is somewhere between the top and bottom of the plate 10.

This leaves a space 22 bounded on the bottom by the plate 16, on the outside by the mold band 18, and on the inside by the periphery of the plate 10 and the periphery of the consolidated center 15a. The top of this space 22 to be filled is somewhat below the level of the shoulder 21. Referring to Figure 4, I now fill this space with a diamond containing ceramic mix 23. I then place the ring 11 inside the mold band 18 upon the shoulder 21, as shown. It will be noted that the height of the ring 11 is the same as that of the plate 10 but the distance from the shoulder 21 to the top of the mold band 18 is slightly less. I now remove the spacing blocks 19 and close the mold to the position shown in Figure 5. The quantity of material 15 and 23, respectively, is selected so that the two parts of the wheel will be pressed to definite, predetermined densities or packings of their constituents, and usually so that the two parts of the wheel will have similar densities of packing, that is, the porosity of the rim and the center will be similar. The closing of the mold to the position shown in Figure 5, however, further presses the consolidated mix 15a simultaneously with the compression of the fill 23, so that the pressed center 15b and the pressed fill 23a are of equal height and consolidated into an integral article which can be readily handled even before it is fired. Such an article is termed a "green" wheel in the abrasive industry.

I now strip the mold band 18, remove the plug 12, and then pick off the plate 16 and the plate 10 and ring 11. I now have a "green" wheel consisting of a non-abrasive center part 15b and an abrasive periphery 23a in an integral piece, with ceramic material throughout capable of being fired in a suitable furnace into an integral non-swelled grinding wheel.

Considering now the materials which I use to form the abrasive periphery 23a and the center or backing 15b, the former contains diamonds while the latter does not; both parts include ceramic materials, and in accordance with the present invention one or both of the parts contains boron, borides, or reduced boron compounds. The use of boron, borides, or oxidizable boron compounds has at least two desirable functions: (1) It prevents detrimental swelling of the abrasive body due to the evolution of certain gases from the material during the burn in a non-oxidizing atmosphere; and (2) it provides at the same time suitable solid granular material for the vitrified bonded framework of the center or backing 15b and desirably also of the periphery 23a. This use of boron, borides, or reduced boron compounds has enabled me to make non-swelled diamond containing abrasive bodies of excellent quality bonded with a vitrified bond matured in the vicinity of 1000° C. or below in a non-oxidizing atmosphere.

Boron and the borides can collectively be termed "reduced boron compounds" or "oxidizable boron compounds." Such reduced boron compounds may in some cases have a minor amount of oxygen, such as an impurity consisting of a small percentage of a borate. Essen-

tially, however, the material that is useful in this invention is a reduced compound having most of the oxygen eliminated. Elementary boron and the borides have, at temperatures of 1000° C. and also considerably below that temperature, a great affinity for oxygen. In other words, boron forms boric oxide  $B_2O_3$  (anhydrous) while the borides form borates. Any boride which is sufficiently stable under ordinary conditions so that it will not decompose with deleterious effects, and which does not volatilize appreciably at 1000° C., may be used in this invention. I have actually used so-called amorphous boron but crystalline varieties could also be used.

I have also used boron carbide  $B_4C$  which was first produced by Raymond R. Ridgway but other boron carbides known prior to Ridgway, such as that reported to be  $B_6C$ , may also be used. I have also used calcium boride  $CaB_6$ . Examples of other borides which may be used are: copper boride,  $Cu_3B_2$ ; barium boride,  $BaB_6$ ; strontium boride,  $SrB_6$ ; beryllium boride; aluminum boride; silicon boride,  $SiB_3$  or  $SiB_6$ ; zirconium boride,  $Zr_3B_4$ ; chromium boride,  $CrB$  or  $Cr_3B_2$ ; molybdenum boride,  $Mo_3B_4$ ; tungsten boride.

The following examples give, as indicated, usable formulae for the peripheral portion 23a or the center 15b.

#### EXAMPLE I

##### Abrasive periphery

|                                                         | Grams  |
|---------------------------------------------------------|--------|
| Diamond abrasive grains, No. 100 grit size              | 0.1579 |
| Vitrifiable bond No. 1                                  | 0.387  |
| Borosilicate glass powder between 90 and 140 grit size  | 0.371  |
| Reduced boron compound, 100 grit size or finer          | 0.162  |
| 4% Glutoline solution as a temporary binder and wettant | 0.094  |

Vitrifiable bond No. 1 is made from 25 parts of Kentucky No. 6 ball clay and 75 parts of a certain frit prepared from a batch of the following composition:

#### TABLE I

##### Frit batch

|                    | Parts |
|--------------------|-------|
| Borax              | 32.2  |
| Boric acid         | 25.4  |
| Flint              | 37.6  |
| Hydrate of alumina | 1.0   |
| Whiting            | 3.8   |

The foregoing ingredients of the frit batch are thoroughly mixed, fused, and quenched to form a frit in the usual manner, which is then pulverized.

#### EXAMPLE II

##### Center or backing

|                                                         | Grams |
|---------------------------------------------------------|-------|
| Vitreous silica, between 100 and 210 grit size          | 0.453 |
| Vitrifiable bond No. 1                                  | 0.565 |
| Reduced boron compound, No. 180 grit size or finer      | 0.346 |
| 4% glutoline solution as a temporary binder and wettant | 0.087 |

## EXAMPLE III

## Center or backing

|                                                         | Grams |
|---------------------------------------------------------|-------|
| Vitreous silica, between 100 to 210 grit size           | 0.297 |
| Borosilicate glass powder, around 90 grit size          | 0.152 |
| Vitrifiable bond No. 2                                  | 0.320 |
| Reduced boron compound, 180 grit size or finer          | 0.595 |
| 4% Glutoline solution as a temporary binder and wettant | 0.087 |

In the foregoing Example III the vitrifiable bond No. 2 is made from 35 parts of Kentucky No. 6 ball clay mixed with 65 parts of the frit of Table I.

## EXAMPLE IV

## Center or backing

|                                                         | Grams |
|---------------------------------------------------------|-------|
| Vitreous Silica, between 100 and 210 grit size          | 0.780 |
| Kentucky No. 6 Ball clay                                | 0.132 |
| Frit of Table I                                         | 0.397 |
| Boron carbide, 180 grit size                            | 0.053 |
| 4% Glutoline solution as a temporary binder and wettant | 0.087 |

The constituents are thoroughly mixed until a damp, pulverulent, screenable, moldable mix is formed.

The borosilicate glass referred to has approximately the following composition:

|                                | Per cent |
|--------------------------------|----------|
| SiO <sub>2</sub>               | 80.5     |
| B <sub>2</sub> O <sub>3</sub>  | 12.9     |
| Al <sub>2</sub> O <sub>3</sub> | 2.2      |
| Na <sub>2</sub> O              | 3.8      |
| K <sub>2</sub> O               | 0.4      |

Relatively high melting borosilicate glasses are preferred.

The calculated chemical composition of the frit used is as follows:

|                                | Per cent |
|--------------------------------|----------|
| Na <sub>2</sub> O              | 7.3      |
| CaO                            | 3.0      |
| Al <sub>2</sub> O <sub>3</sub> | 0.9      |
| B <sub>2</sub> O <sub>3</sub>  | 36.4     |
| SiO <sub>2</sub>               | 52.4     |

After the "green" wheels are formed, as already described, they are placed in a suitable furnace and burned in a non-oxidizing atmosphere, preferably an atmosphere of nitrogen, which I have found to be very effective. Some atmospheres favor the wetting of the diamonds by the vitrifiable bond more than others. Nitrogen I have found to be particularly effective, or at least nitrogen does not inhibit the wetting of the diamonds to any considerable extent. In order to purify it and eliminate all possible traces of oxygen, the nitrogen should be passed through concentrated sulphuric acid and over a red hot copper gauze. The preferred vitrifying conditions constitute a temperature of around 950° C. maintained for four and one-half hours.

A vitrified bonded supporting center or back made solely of materials which are non-reactive toward the furnace atmosphere is apt to swell objectionably when burned even in a non-oxidizing atmosphere due to the evolution of gas from its constituent materials. This swelling may seriously disturb the structure of portions of the peripheral diamond containing rim which are adjacent to the supporting center. I have found

that the use of boron, such as amorphous boron, or borides such as those herein mentioned, as a whole or part of the granular constituents of the central supporting disk or backing obviates this swelling satisfactorily, and at the same time the reduced boron compound provides a suitable material for the vitrified bonded framework of the supporting center. Here also, as in the diamond containing rim, the reduced boron compound serves the dual function of controlling the swelling in a non-oxidizing atmosphere and of serving as a structural element of the center.

It will thus be seen that there has been provided by this invention an article and a method in which the various objects hereinabove set forth together with many thoroughly practical advantages are successfully achieved. As various possible embodiments might be made of the mechanical features of the above invention and as the art herein described might be varied in various parts, all without departing from the scope of the invention, it is to be understood that all matter hereinbefore set forth or shown in the accompanying drawing is to be interpreted as illustrative and not in a limiting sense.

I claim:

1. A vitrified-bonded abrasive article comprising the bonded reaction product, as a result of firing, of a mix that comprises abrasive grains, 30 granules of an oxidizable boron compound, and vitrifiable bond, granules of said compound being present in the vitrified product in an amount, exclusive of any oxidation product formed during firing as a result of oxidation of some of said 35 compound, to constitute a substantial proportion of the volume of the vitrified article and being bonded by, and distributed in said amount throughout, the vitrified bond thereby to reinforce the bond and to form with the vitrified 40 bond a built-up framework of which the granules of said compound, in said substantial proportion, are material structural parts, said abrasive grains being distributed throughout, and supported by, said build-up framework and bonded therein by the vitrified bond of said framework.

2. A vitrified bonded abrasive article having a unitary body comprising a vitrified-bonded abrasive portion and a vitrified-bonded backing portion, and being the unitary bonded reaction 50 product as a result of firing together two mixes, one of which comprises abrasive grains and vitrifiable bond and the other of which comprises vitrifiable bond and granules of an oxidizable boron compound, granules of said oxidizable 55 boron compound being present in the vitrified-bonded backing portion in an amount, exclusive of any oxidation product formed during firing as a result of oxidation of some of said compound, to constitute a substantial proportion structurally of the said backing portion and the said granules being bonded by, and distributed in said substantial proportion throughout the vitrified bond of said backing portion to form a built-up framework of which said oxidizable compound granules are in said amount material structural parts to thereby constitute said backing portion to support said abrasive portion.

3. A vitrified bonded abrasive article having a unitary body comprising a vitrified-bonded abrasive portion and a vitrified-bonded backing portion, and being the unitary bonded reaction product as a result of firing together two mixes, one of which comprises abrasive grains and vitrifiable bond and granules of an oxidizable boron compound and the other of which comprises vitrifi-

able bond and granules of an oxidizable boron compound, granules of said oxidizable boron compound being present in each of said portions in an amount, exclusive of any oxidation product formed during firing as a result of oxidation of some of said compound, to constitute a substantial proportion structurally of said abrasive portion and of said backing portion and the said granules being in each portion bonded by, and distributed in said substantial proportion throughout, the vitrified bond in each portion to form in each a built-up framework of which said oxidizable compound granules are in said amount material structural parts, said abrasive grains being distributed throughout, and supported by, said built-up framework of the abrasive portion and bonded therein by the vitrified bond in said portion, the built-up framework of the backing portion constituting a support for said abrasive portion.

4. A vitrified-bonded abrasive article having a unitary body comprising a vitrified-bonded abrasive portion and a vitrified-bonded backing portion, and being the unitary bonded reaction prod-

uct as a result of firing together two mixes, one of which comprises abrasive grains and vitrifiable bond and the other of which comprises vitrifiable bond and granules of an oxidizable boron compound and body material comprising granules of vitreous silica, granules of said oxidizable boron compound and granules of said vitreous silica being present in the vitrified-bonded backing portion in an amount, exclusive of any oxidation product formed during firing as a result of oxidation of some of said compound, to constitute a substantial proportion structurally of the said backing portion and the said granules of vitreous silica being bonded by, and distributed in said substantial proportion throughout, the vitrified bond of said backing portion to form a built-up framework of which said oxidizable compound granules and vitreous silica granules are in said amount material structural parts to thereby constitute said backing portion to support said abrasive portion.

ROBERT H. LOMBARD.